

Aug. 3, 1937.

H. DANNENBERG ET AL

2,089,159

MANUFACTURE OF ARTIFICIAL THREADS

Filed March 8, 1934

3 Sheets-Sheet 1

Fig. 2



Fig. 1



Fig. 1a



By

Inventors:  
Hans Dannenberg,  
Emil Hubert,  
Attorneys  
Potter, Pierce & Schaffler.

Aug. 3, 1937.

H. DANNENBERG ET AL

2,089,159

MANUFACTURE OF ARTIFICIAL THREADS

Filed March 8, 1934

3 Sheets-Sheet 2

*Fig. 3*



*Fig. 4*



Inventors:  
Hans Dannenberq,  
Emil Hubert,  
Attorneys  
Potter, Pierce & Scheffler.

Aug. 3, 1937.

H. DANNENBERG ET AL

2,089,159

MANUFACTURE OF ARTIFICIAL THREADS

Filed March 8, 1934

3 Sheets-Sheet 3

*Fig. 5*



*Fig. 6*



*Fig. 7.*



By

Attorneys

Inventors:

Hans Dannenberq,

Emil Hubert,

Potter, Pierce & Schaffler.

## UNITED STATES PATENT OFFICE

2,089,159

## MANUFACTURE OF ARTIFICIAL THREADS

Hans Dannenber, Dessau, and Emil Hubert, Dessau-Ziebigk, Germany, assignors to I. G. Farbenindustrie Aktiengesellschaft, Frankfort-on-the-Main, Germany

Application March 8, 1934, Serial No. 714,721  
In Germany March 9, 1933

8 Claims. (CL. 18—8)

Our present invention relates to the art of manufacturing artificial threads.

One of its objects is to provide a new process of manufacturing artificial silk and more particularly to a new process of assembling spun threads to an efficient package or cake for further treatment. Another object is the package of threads obtained by our new process. Further objects will be seen from the detailed specification following hereafter. Reference is made to the accompanying drawings in which Figs. 1 and 1a illustrate the spinning process, Figs. 2, 3 and 4 show the manner in which the thread is deposited, Figs. 5 and 6 show conventional view of a finished package or cake. Fig. 7 is a detailed vertical cross-sectional view of a preferred form of the mechanism for imparting movement to table 5 of Fig. 1.

It is known to produce artificial silk by causing a thread spun in the usual way into a spinning bath and drawn off by a galette rotating at the required speed of draft to fall freely into a slowly rotating box in which the thread is collected.

In this process a regular deposition of the thread within the box is realized by imparting to the box a revolving and a reciprocating movement. In this manner the threads are piled crosswise in the form of loose loops which, when the box is filled, are reeled from the box to form hanks which may be after-treated in this form.

As artificial silk, in many cases, is no longer delivered to the consumer by the manufacturer in the form of hanks, but in a wound form, it is no longer desirable to after-treat artificial silk in hank-form. The actual state of art, for avoiding any superfluous operation, requires the filaments to be after-treated in the form in which they were spun. This is not possible with the loose layers of threads, such as they are produced in slowly rotating spinning pots as described above. The loose layers suffer so much relative displacement by the washing and after-treating liquids that reeling off the content of the spinning pot becomes impossible in most cases. In any case the threads are rendered highly unfit for winding.

According to this invention we have found that it is possible to pile up the spun thread in form of a solid cake capable of retaining its form in handling it in the washing and after-treatment operations and which needs no support at all neither during its production nor in handling it as aforesaid. The cake produced in this manner may be washed and after treated in the same way as a centrifugal cake, while freely lying on

a plate, or hanging on rods or arranged in any suitable manner, without incurring displacement of the threads or impairing their capacity of being wound.

The improvement is attained in the following way:

Referring to Fig. 1, the thread 1 issuing from the nozzle 2 and coagulated in the spinning bath 3 is guided around the galette 4 and the thread falls from the galette 4 on the plate 5, which performs a rotary movement and an additional movement, for instance a reciprocating or an eccentric movement. The ratio between the period of the rotary movement and the period of the additional movement must be so adjusted that the layers of threads deposited on the plate form a regular system of crossings in which each thread has its determined position. It is particularly advantageous to wind the threads in such a manner that the windings lie closely side by side at a distance of about 2 to 5 mm. from each other. Fig. 3 shows the form of the windings which are deposited closely to each other and are helically piled up to form the cake. Under these conditions the layers of thread form a body occupying a minimum of space and the cake being therefore very solid. In other words, the package of threads conserving its form in the usual treatment with liquid is obtained according to the present invention by a method of winding the threads so as to save space. Fig. 4 shows for instance, diagrammatically the crossing of the thread in one layer. This figure has been obtained by covering with a paper a rotating plate to which an additional reciprocating movement has been imparted by a planetary gear and pressing a writing device, for instance, a pencil against the paper. The construction of a planetary gearing for imparting motion to the spinning box 5 is represented on a larger scale in Fig. 7. The shaft 11 drives the shaft 12 through the gear wheels 13 and 14. Wheel 14 has an eccentrically mounted bushing 15 in which rotates the planetary shaft 16. On top of this shaft there is mounted the revolving plate (spinning box) 5, whereas at its lower end there is keyed a toothed wheel 17 which engages a stationary toothed wheel 18 carried by the base plate 19. When 14 and 16 turn about 12, 17 rotates by gearing with 18, and 16 and 5 turn on the axis of 16. This rotation is the main movement, whereas the rotation on the axis of 16 and 12 constitutes the additional circular movement.

The number of teeth of the toothed wheels 17 55

and 18 must be so chosen that the desired crossing of the threads is obtained which realizes the greatest economy of space and yields solid spinning cakes. The following data are given 5 as an example of suitable planetary gearing:

Number of teeth of 17..... 24  
 Number of teeth of 18..... 25  
 Eccentricity 12-14..... 24.5 mm.  
 10 Number of revolutions of 12 112.3 revolutions  
 about 16. per minute  
 Number of revolutions of 16 55 revolutions  
 about 12. per minute

The receiving member for the threads, in simple cases, is constructed in the form of a level, plate-shaped disk. There may, however, also be employed a conical or otherwise suitably profiled disk. Finally there may also be used a spinning box of any suitable size.

20 In order to obtain a completely unobjectionable package of threads two further conditions must be considered. The first condition is that the additional movement of the plate must not be too quick. Preferably the additional movement corresponds approximately with two revolutions of the plate that is to say one reciprocation must occur on somewhat more or less than two revolutions of the plate in which case the thread is deposited on the plate in double loops as shown in 25 Fig. 2. If one reciprocating would occur on exactly one revolution or a whole number of revolutions an unserviceable cake or no cake at all is formed because in this case all loops would be deposited at the same place. The highest admissible speed is that at which one reciprocating movement takes place on every half turn of the plate. If the reciprocating additional movement is slower than the speed of the plate the thread is deposited on the plate in form of loops having 30 a curvature which always appears concave when viewed from the center of the cake. If the reciprocating additional movement is quicker there are formed loops having varying curvature in such a manner that the curvature of the loops when 35 viewed from the center of the cake alternately appears convex and concave. This form of loop is not favorable and yields unserviceable cakes when the reciprocating movement is quicker than the above mentioned limit of more than one reciprocating on half a revolution. A too quick reciprocating movement involves the further difficulty that the thread is no longer capable to follow the movement of the support with the required 40 accuracy; in this case the thread comes not to lie at the intended place so that only a loose accumulation of threads occurs.

The second condition which must be considered for the production of an unobjectionable package of threads, is to stabilize the pendulum swingings which invariably occur at the freely hanging part of the thread. The cause for this swinging will now be explained with reference to Fig. 2. The freely hanging thread is received by the plate 5 at 6, the speed of the thread being equal 45 to the peripheral speed of point 6. However, by the additional movement the thread is guided alternately outwards, towards the path of point 7, and inwards, towards the path of point 8. Points 50 7 and 8, however, run at a higher and a lower speed than point 6. The thread, therefore, falls on a support which is moved alternately more swiftly and more slowly than the constant speed, at which the thread is supplied and, therefore, the thread is alternately pulled along or pushed 55 back. The hanging thread, therefore, does not

move on the path between the points 7 and 8, but, for instance, on the path between the points 9 and 10. Therefore the thread performs considerable pendulum swingings about the point 11 (see Fig. 1) at which the thread leaves the galette. In consequence the additional movement is the cause of these pendulum swingings.

As it has been found these pendulum swingings cause troubles only when taking an irregular course. In this case the winding system becomes less accurate. Furthermore, the thread easily forms small loops or knots or is deposited across the packages at its points of reversion. Completely uniform oscillations, however, do not interfere with the accuracy of the windings. The production of such uniform oscillations was realized by profiting of the resonance phenomena, which as is known occurs with any kind of oscillation. The free part of the thread which oscillates has a natural oscillation which depends on the weight of the thread, on the weight of the portions of the spinning bath adhering to the thread and on its dimensions. If the time of the natural oscillation corresponds with the period of the additional movement of the rotating plate that is with the time of one reciprocation, resonance between the two is produced that is to say the thread oscillates uniformly and quickly without trembling or shaking and the formation of a regularly wound and solid cake occurs. Resonance is also produced if the time of oscillation and the time of revolution are in a ratio of 1:2, 1:3, 2:1, etc., that is to say in the case of a so-called harmonic.

While the mechanism preferably adopted in the process according to the present invention for imparting to the spinning box both a reciprocating and a rotary movement about its shaft is the planetary gear disclosed in Fig. 7, in principle any device for effecting a rotary movement and an additional reciprocating movement, subject to the above condition, is suitable for use with the rotary plate for depositing the threads.

The following examples illustrate the invention:

*Example 1.*—For a viscose thread with a titer of 180 den. prepared in a spinning bath having a specific weight of 1.4 and spun at a speed of 60 m. per minute, the resonance effect is obtained by giving the measures *a*, *b*, *c*, *d* of Figs. 1 and 1a the following values:

*a*=725 mm.  
*b*= 95 mm.  
*c*= 80 mm.  
*d*= 50 mm.

The plate is rotated at a speed of 112.3 revolutions per minute, and makes 55 reciprocations per minute. The cake obtained after 6 hours' spinning had the following dimensions:

| Thread package      | Freshly spun<br>acid moist | Washed and<br>dried |
|---------------------|----------------------------|---------------------|
| Outer diameter..... | 190 mm.....                | 178 mm.....         |
| Inner diameter..... | 100 mm.....                | 78 mm.....          |
| Middle height.....  | 92 mm.....                 | 51 mm.....          |
| Weight.....         | 1,270 grams.....           | 400 grams.....      |
| Density.....        | 0.723 gram/cc.....         | 0.360 gram/cc.....  |

Total titer..... 180 deniers  
 Single titer..... 5 deniers  
 Length of thread..... 20,000 meters

*Example 2.*—When spinning a viscose thread having a titer of 300 deniers at the same speed

in a spinning bath of the same specific weight the values of  $a$ ,  $b$ ,  $c$  and  $d$  are the following:

$a=780$  mm.  
 $b=150$  mm.  
 $c=70$  mm.  
 $d=50$  mm.

The plate is rotated at a speed of 112.3 revolutions per minute, and makes 55 reciprocations per minute. The cake obtained after 6 hours' spinning had the following dimensions:

| Thread package            | Freshly spun<br>acid moist | Washed and<br>dried |
|---------------------------|----------------------------|---------------------|
| Outer circumference.....  | 660 mm.....                | 625 mm.....         |
| Outer diameter.....       | 210 mm.....                | 198 mm.....         |
| Inner circumference.....  | 375 mm.....                | 277 mm.....         |
| Inner diameter.....       | 120 mm.....                | 88 mm.....          |
| Middle height.....        | 135 mm.....                | 75 mm.....          |
| Volume.....               | 3,150 cc.....              | 1,853 cc.....       |
| Weight.....               | 2,250 grams.....           | 660 grams.....      |
| Density.....              | 0.715 gram/cc.....         | 0.356 gram/cc.....  |
| Total titer.....          | 300 deniers                |                     |
| Single titer.....         |                            | 5 deniers           |
| Length of the thread..... | 20,000 meters              |                     |

Figs. 5 and 6 show a finished cake. As seen from these figures in practice the inner and the outer border of the cake may show a slight deformation. The outer, upper edge of the cake is generally somewhat rounded whereas the inner, upper border may be somewhat raised. The walls of the cake are perfectly smooth and vertical on the plate.

The diameter of the cake is determined by the speed at which the plate is rotated and the speed at which the thread is supplied. The mean diameter of the cake (see the dotted line in Fig. 2) is equal to

$$40 \quad \text{speed at which the thread is supplied} \\ \pi \cdot \text{number of revolutions of the plate}$$

The breadth of the cake is approximately equal to the width of the reciprocating movement. The density of the dry cake may vary between 0.2 to 45 0.5 gram/cc. as has been found, without however limiting our invention to these values.

According to our invention there may be produced packages having a very great length of thread of about 20,000 meters or 30,000 meters 50 which varies with the titer of the spun thread. The advantage of the present invention over the hitherto used bobbin spinning system and centrifugal spinning results from the following table:

| 55                                  | Bobbin spinning                      | Centrifugal<br>spinning              | Plate spinning |
|-------------------------------------|--------------------------------------|--------------------------------------|----------------|
| 100 grams.....<br>6,000 meters..... | 165 grams.....<br>10,000 meters..... | 500 grams.....<br>30,000 meters..... |                |

60 which is drafted for a titer of 150 deniers.

The process according to this invention obviously is not limited to spinning viscose silk as shown in the examples but is adapted for spinning spinning solutions according to the wet spinning process quite generally. Thus, there may be spun solutions of cellulose acetate or another cellulose derivative or there may be spun solutions of fibroin according to the wet spinning 65 process.

70 What we claim is:

1. A process of producing artificial silk which comprises ejecting a spinning solution into a precipitating bath, guiding the coagulated thread 75 around a rotating galette, causing the thread to

fall freely upon a plate, rotating said plate at a speed so that a point of the plate at a substantial distance from the center of rotation and from the periphery of said plate has the same peripheral velocity as said galette, giving the plate 5 an additional reciprocating movement so that at most one reciprocation occurs on half a revolution of the plate and adjusting the free length of the thread between the point at which the thread leaves the galette and the point at which the thread falls on the rotating plate so that the 10 natural vibrations of the thread are in resonance with the reciprocating movement, whereby a cake which needs no support is obtained.

2. A process of producing artificial silk which 15 comprises ejecting a spinning solution into a precipitating bath, guiding the coagulated thread around a rotating galette, causing the thread to fall freely upon a plate, rotating said plate at a speed so that a point of the plate at a substantial distance from the center of rotation and from the periphery of said plate has the same peripheral velocity as said galette, giving the plate an additional reciprocating movement so that at most one reciprocation occurs on approximately 20 two revolutions of the plate and adjusting the free length of the thread between the point at which the thread leaves the galette and the point at which the thread falls on the rotating plate so that the natural vibrations of the thread are in 25 resonance with the reciprocating movement, whereby a cake which needs no support is obtained.

3. An annular self-supporting package of 30 artificial threads comprising double loops of thread helically arranged around an inner free space, the free space being inside both loops and the center of curvature of the loops appearing always concave when viewed from the center of the cake, said package having a density in the dry state of 0.2 to 0.5 gram/cc., each loop being slightly displaced from the next, and the loops following each other to form one layer lying in substantially the same plane at a right angle to the axis of the annulus, said package being substantially identical with that produced by the process of 35 claim 1.

4. A device for spinning artificial silk thread and assembling the spun thread into a package, 40 which comprises a spinning nozzle, a galette for drawing off a thread emanating from said spinning nozzle, a receiving member for collecting the thread delivered by said galette, and means for assembling the thread upon said receiving member in the form of a self-supporting winding, said 45 assembling means including means for rotating the receiving member in a plane normal to the axle of said receiving member and means for imparting to the receiving member an additional reciprocating movement so that at most one reciprocation occurs during a half revolution of the receiving member, in the plane of the thread-receiving surface thereof, the receiving member being arranged at a distance from the galette such that the natural vibrations of the thread falling on said receiving member are in resonance with the reciprocating movement of said receiving member.

5. A device for spinning artificial silk thread and assembling the spun thread into a package, 50 as defined in claim 4, characterized in that the reciprocating movement is imparted by reciprocating means.

6. A device for spinning artificial silk thread and assembling the spun thread into a package, 55

- which comprises a spinning nozzle, a galette for drawing off a thread emanating from said spinning nozzle, a receiving member for collecting the thread delivered by said galette, and means 5 for assembling the thread upon said receiving member in the form of a self-supporting winding, said assembling means including means for imparting to the receiving member a planetary movement in the plane of the thread receiving 10 surface thereof, the receiving member being arranged at a distance from the galette such that the natural vibrations of the thread falling on said receiving member are in resonance with the cyclic movement of said receiving member.
- 15 7. A device for spinning artificial silk thread and assembling the spun thread into a package, as defined in claim 4, characterized in that the receiving member is a plate.

8. An annular self-supporting package of arti-

ficial threads comprising double loops of thread helically arranged around an inner free space, the free space being inside both loops and the center of curvature of the loops appearing always concave when viewed from the center of the package, said package having a density in the dry state of 0.2 to 0.5 grams per c. c. and comprising 20,000 meters of the washed and dried thread in a volume of about 6 c. c. multiplied by the titre of the fiber, each loop being slightly 10 displaced from the next and the loops following each other to form one layer lying in substantially the same plane at a right angle to the axis of the annulum, said package being substantially identical with that produced by the process 15 of claim 1.

HANS DANNENBERG.

EMIL HUBERT.